

## UNITED STATES PATENT OFFICE

2,242,225

## SPINNING PROCESS

Rudolph S. Bley, Elizabethton, Tenn., assignor to  
 North American Rayon Corporation, New York,  
 N. Y., a corporation of Delaware

No Drawing. Application December 2, 1937,  
 Serial No. 177,822

13 Claims. (Cl. 18—54)

In the manufacture of cellulosic products, such as filaments, threads, and the like, a viscose solution is continuously extruded through the minute orifices of a spinneret into a coagulating or setting bath (spin bath). However, since the introduction of the viscose process great troubles have been and are still experienced as far as continuous spinning is concerned due to impurities, such as, for example, precipitated cellulose particles, sulphur and resin particles, zinc compounds, etc., present in either the viscose solution or the spin bath. These impurities gradually contaminate the spinnerets, clog and reduce the widths of the spinneret holes with the result that filaments of uneven thickness are obtained. If the contamination of the spinnerets and the clogging of their holes proceeds the individual filaments start to tear and occasion interruption of the spinning process.

By experimentation, I have found that the contamination of spinnerets and the clogging of spinneret holes may be overcome by spinning viscose solutions in the presence of cation-active compounds, these compounds being produced by condensing a halogenated petroleum or a halogenated petroleum constituent containing at least one hydrocarbon having a chain of eight or more carbon atoms with an organic sulphide, selected from the group consisting of dialkyl sulphides, diaryl sulphides and alkyl-aryl sulphides under substantially anhydrous conditions.

Petroleum consists of complex mixtures of hydrocarbons concerning the chemical nature of which there is very little information, although there are indications that all of these materials contain members of the methane series, the polymethylene series and the benzene series of hydrocarbons. The difference between petroleums of various sources resides in the proportions of the different types of hydrocarbons and in the chemical nature and amounts of their impurities. Pennsylvania oil, for example, contains a large proportion of methane hydrocarbons and practically no impurities of sulphur or nitrogen compounds. About thirty hydrocarbons have been isolated and identified with certainty. Distillation is the principal method in separating petroleum into useful components. The distilled fractions from crude petroleum are casinghead gasoline, gasoline, kerosene, gas oil and lighter lubricating oils (" neutrals"). The residues from such distillation supply most of the lubricating oils (" bright stock"), petrolatum in pasty or liquid form and either paraffin wax or petroleum pitch, depending upon the nature

of the crude petroleum. Kerosene is any mixture of hydrocarbons which is not volatile enough for use in explosion motors. Cracked gasolines are rich in olefins and diolefins. Paraffin wax was originally obtained from tars from the distillation of wood, peat, and lignite, but is now obtained from petroleum, and especially from Pennsylvania paraffin-base oils. Little information is available about the composition of paraffin waxes except that it consists mainly of higher alkanes and only small amounts of the normal compounds. Petrolatum (vaseline) is a pasty mixture of hydrocarbons similar to paraffin while liquid petrolatum is a high boiling petroleum distillate. Ozokerite is a natural paraffin wax originating in Galicia; in bleached form it is termed "ceresin." All of these petroleum hydrocarbons may be halogenated in conventional manner in the presence or absence of catalysts to form halogenated hydrocarbon mixtures adapted to be condensed with the tertiary bases and organic sulphides, set forth above. The materials, i. e., crude petroleums, gasolines, kerosenes, lubricating oils, pasty petrolatums, liquid petrolatums and paraffin waxes, to be halogenated may first be dissolved in carbon tetrachloride, etc., and subsequently chlorine, bromine, etc., in gaseous form introduced therein until the heat of reaction abates. Halogenated compounds, containing about 25 to 40% of halogen may be obtained in this manner. However, upon prolonging the introduction of halogens, compounds may be obtained containing up to about 75% of a halogen, and it is to be noted that the boiling or fusing points of the raw materials are either lowered or raised by halogenation. Hydrochloric acid, hydrobromic acid, etc., formed during this reaction must be removed, preferably by neutralization. Catalysts, such as iron, etc., may be added to the mixtures to accelerate halogenation. Halogenation will also proceed more rapidly by carrying out the reaction under the influence of ultraviolet rays. The halogenation may also be performed in accordance with processes disclosed, for example, in U. S. Patent #989,225 to Blakeman of April 11, 1911; U. S. Patent #1,246,810 to Ellis of November 13, 1917; U. S. Patent #1,432,761 to Koch of October 24, 1922; etc. Chlorinated paraffin wax, sold under the trademark of "Chlorafin" is a very suitable raw material for my process.

Organic sulphides capable of being condensed with the halogenated, hydrocarbonaceous materials set forth above are dialkyl sulphides,

diaryl sulphides and alkyl-aryl sulphides, having the following structure:



in which  $R_1$  and  $R_2$  represent monovalent aliphatic (alkyl) or aromatic (aryl) radicals. Examples of such organic sulphides are dimethyl sulphide, diethyl sulphide, methyl-ethyl sulphide, methyl-propyl sulphide, dibutyl sulphide, methyl-benzyl sulphide, propyl-ethyl sulphide, dibenzyl sulphide, diphenyl sulphide, etc.

Thus, by condensing an organic sulphide with a halogenated, hydrocarbonaceous material of the aforementioned group, sulphonium halides are obtained, having the structure:



in which  $P$  represents a petroleum hydrocarbon chain. If  $P$  is a chain containing eight or more carbon atoms the sulphonium halide becomes cation-active and an incrustation inhibitor. Cation-active compounds are surface-active compounds which carry in the cation a hydrocarbon chain having eight or more carbon atoms. They are particularly advantageous because they may be used in neutral (salt), alkaline and acidic aqueous solutions, and also in hard water. In contradistinction to cation-active compounds, anion-active compounds are surface-active compounds which carry in the anion a more or less extended hydrocarbon chain (fat chain). They flocculate in neutral (salt), alkaline and acidic aqueous solutions, and also in hard water. Common soaps, sulphonated oils, salts of sulphonated fatty acids, etc., are examples of anion-active compounds, and they are unable to prevent the incrustation of spinnerets and spinneret holes. These incrustation inhibitors are prepared by heating a halogenated hydrocarbonaceous material selected from the group consisting of crude petroleums, gasolines, kerosenes, lubricating oils, pasty petrolatums, liquid petrolatums and paraffin waxes by heating under reflux until condensation is completed. About 0.4 to 1.0 gram of the condensation products are added to one liter of a viscose solution of conventional cellulose content and maturity. This solution is then spun into a conventional, acid spin bath, such as, for example, a glucose bath, a magnesium-zinc bath, etc. The spinnerets and spinneret holes remain clean on prolonged spinning in comparison with the spin bath free from cation-active compounds. Any dialkyl sulphide, diaryl sulphide or alkylaryl sulphide may be used in the condensation, which may be carried out at any temperature at which the two reactants and the sulphonium halide remain stable.

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

588

590

595

598

600

605

610

615

620

625

630

635

640

645

650

655

660

665

670

675

680

685

690

695

700

705

710

715

720

725

730

735

740

745

750

755

760

765

770

775

780

785

790

795

800

805

810

815

818

820

825

830

835

838

840

845

850

855

858

860

865

870

875

880

885

890

895

900

905

910

915

918

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1138

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

lustre, etc., of regenerated cellulose produced therefrom or therein, respectively, remain practically unaltered. Upon increasing the amount of incrustation inhibitor in a given viscose solution or spin bath, the regenerated cellulose produced therefrom or therein, respectively, may alter its physical characteristics, i. e., it may acquire a soft lustre, become more plastic, lose part of its original strength, etc. For such reasons, the amounts of such compounds to be added to viscose solutions or spin baths control the physical properties of the finished cellulosic products. In other words, these additions are critical and their amounts must be predetermined by experimentation. Additions of about 0.4 to 1.0 gram per liter of viscose or spin bath are insufficient to substantially alter the physical characteristics of regenerated cellulose although they allow continuous spinning for long periods of time.

Although these cation-active sulphonium compounds improve the spinning properties of any conventional viscose solution or any spin bath known in the art, I have found that they are especially valuable additions to zinc-bearing baths which tend to interrupt spinning, i. e., spin baths containing zinc compounds, such as, for example, zinc sulphate.

#### Example 1

Ethyl-methyl sulphide is condensed with a halogenated, hydrocarbonaceous material selected from the group consisting of crude petroleums, kerosenes, gasolines, lubricating oils, pasty petrolatums, liquid petrolatums and paraffin waxes by heating under reflux until condensation is completed. About 0.4 to 1.0 gram of the condensation products are added to one liter of a viscose solution of conventional cellulose content and maturity. This solution is then spun into a conventional, acid spin bath, such as, for example, a glucose bath, a magnesium-zinc bath, etc. The spinnerets and spinneret holes remain clean on prolonged spinning in comparison with the spin bath free from cation-active compounds. Any dialkyl sulphide, diaryl sulphide or alkylaryl sulphide may be used in the condensation, which may be carried out at any temperature at which the two reactants and the sulphonium halide remain stable.

#### Example 2

An alkyl-aryl sulphide, a dialkyl sulphide or a diaryl sulphide, such as, for example, dibenzyl sulphide is condensed with a halogenated paraffin wax in the presence of an inert solvent, such as, for example, benzene, etc., under substantially anhydrous conditions. A conventional viscose solution is extruded through fine orifices of a spinneret of a precious metal into an acid spin bath, this bath containing sulphuric acid, sodium sulphate, ammonium sulphate and zinc sulphate plus about 0.05% by weight of a cation-active substance set forth above. Spinning irregularities and difficulties are substantially overcome while without this inhibitor spinning is interrupted after a very short period of time. These inhibitors are especially suitable for continuous spinning processes using sulphuric acid-zinc sulphate baths. These sulphides may be condensed with any halogenated, hydrocarbonaceous material of the group set forth above.

#### Example 3

Cation-active condensation products are added to both the viscose solutions and the spin baths

to allow continuous formation of lustrous or soft-lustre viscose products.

Although these examples will serve to illustrate the present invention, I do not wish to be limited to the inhibitors and concentrations thereof recited therein, since I may use any cation-active sulphonium compound of the group set forth above and vary the physical characteristics of regenerated cellulose by varying their amounts in viscose solutions and/or spin baths, provided these inhibitors are sufficiently soluble in viscose solutions and/or spin baths to furnish cations therein.

Modifications of my invention will readily be recognized by those skilled in the art, and I desire to include all such modifications and variations coming within the scope of the appended claims.

I claim:

1. A spin bath, adapted for use in the manufacture of regenerated cellulose, containing about 0.4 to 1.0 gram per liter of a cation-active condensation product of a halogenated hydrocarbonaceous material selected from the group consisting of crude petroleums, gasolines, kerosenes, lubricating oils, pasty petrolatums, liquid petrolatums and paraffin waxes and an organic sulphide, said condensation product being sufficiently soluble and stable in said setting bath to become cation-active therein.

2. A spin bath, adapted for use in the manufacture of regenerated cellulose, containing about 0.4 to 1.0 gram per liter of a cation-active condensation product of a halogenated hydrocarbonaceous material selected from the group consisting of crude petroleums, gasolines, kerosenes, lubricating oils, pasty petrolatums, liquid petrolatums and paraffin waxes and a dialkyl sulphide, said condensation product being sufficiently soluble and stable in said setting bath to become cation-active therein.

3. A spin bath, adapted for use in the manufacture of regenerated cellulose, containing about 0.4 to 1.0 gram per liter of a cation-active condensation product of a halogenated hydrocarbonaceous material selected from the group consisting of crude petroleums, gasolines, kerosenes, lubricating oils, pasty petrolatums, liquid petrolatums and paraffin waxes and an alkyl-aryl sulphide, said condensation product being sufficiently soluble and stable in said setting bath to become cation-active therein.

4. A spin bath, adapted for use in the manufacture of regenerated cellulose, containing about 0.4 to 1.0 gram per liter of a cation-active condensation product of a halogenated hydrocarbonaceous material selected from the group consisting of crude petroleums, gasolines, kerosenes, lubricating oils, pasty petrolatums, liquid petrolatums and paraffin waxes and a diaryl sulphide, said condensation product being sufficiently soluble and stable in said setting bath to become cation-active therein.

5. A spin bath, adapted for use in the manufacture of regenerated cellulose, containing about 0.4 to 1.0 gram per liter of a cation-active condensation product of a chlorinated paraffin wax and an ethyl-methyl sulphide.

6. A spin bath adapted to be used in the manufacture of regenerated cellulose from viscose solutions comprising sulphuric acid, a water-soluble zinc compound and about 0.4 to 1.0 gram per liter of said bath of a cation-active condensation product of a halogenated hydrocarbonaceous material selected from the group consisting of crude

petroleums, gasolines, kerosenes, lubricating oils, pasty petrolatums, liquid petrolatums and paraffin waxes with an organic sulphide, said condensation product being sufficiently soluble and stable in said bath to become cation-active therein.

7. A spin bath adapted to be used in the manufacture of regenerated cellulose from viscose solutions comprising sulphuric acid, a water-soluble zinc compound and about 0.4 to 1.0 gram per liter of said bath of a cation-active condensation product of a halogenated hydrocarbonaceous material selected from the group consisting of crude petroleums, gasolines, kerosenes, lubricating oils, pasty petrolatums, liquid petrolatums and paraffin waxes with a dialkyl sulphide, said condensation product being sufficiently soluble and stable in said bath to become cation-active therein.

8. A spin bath adapted to be used in the manufacture of regenerated cellulose from viscose solutions comprising sulphuric acid, a water-soluble zinc compound and about 0.4 to 1.0 gram per liter of said bath of a cation-active condensation product of a halogenated hydrocarbonaceous material selected from the group consisting of crude petroleums, gasolines, kerosenes, lubricating oils, pasty petrolatums, liquid petrolatums and paraffin waxes with an alkyl-aryl sulphide, said condensation product being sufficiently soluble and stable in said bath to become cation-active therein.

9. A spin bath adapted to be used in the manufacture of regenerated cellulose from viscose solutions comprising sulphuric acid, a water-soluble zinc compound and about 0.4 to 1.0 gram per liter of said bath of a cation-active condensation product of a halogenated hydrocarbonaceous material selected from the group consisting of crude petroleums, gasolines, kerosenes, lubricating oils, pasty petrolatums, liquid petrolatums and paraffin waxes with a diaryl sulphide, said condensation product being sufficiently soluble and stable in said bath to become cation-active therein.

10. A spin bath adapted to be used in the manufacture of regenerated cellulose from viscose solutions comprising sulphuric acid, a water-soluble zinc compound and about 0.4 to 1.0 gram per liter of said bath of a cation-active condensation product of a chlorinated paraffin wax and ethyl-methyl sulphide.

11. A spin bath adapted to be used in the manufacture of regenerated cellulose from viscose solutions comprising sulphuric acid, a water-soluble zinc compound and a cation-active condensation product of a halogenated hydrocarbonaceous material selected from the group consisting of crude petroleums, gasolines, kerosenes, lubricating oils, pasty petrolatums, liquid petrolatums and paraffin waxes with an organic sulphide, said condensation product being sufficiently soluble and stable in said bath to become cation-active therein.

12. A spin bath adapted to be used in the manufacture of regenerated cellulose from viscose solutions comprising sulphuric acid, a water-soluble zinc compound and a cation-active condensation product of a halogenated hydrocarbonaceous material selected from the group consisting of crude petroleums, gasolines, kerosenes, lubricating oils, pasty petrolatums, liquid petrolatums and paraffin waxes with a dialkyl sulphide, said condensation product being suffi-

ciently soluble and stable in said bath to become cation-active therein.

13. A spin bath adapted to be used in the manufacture of regenerated cellulose from viscose solutions comprising sulphuric acid, a water soluble zinc compound and a cation-active condensation product of a halogenated hydrocarbonaceous material selected from the group con-

sisting of crude petroleum, gasolines, kerosenes, lubricating oils, pasty petrolatums, liquid petrolatums, and paraffin waxes with an alkyl-aryl sulphide, said condensation product being sufficiently soluble and stable in said bath to become cation-active therein.

RUDOLPH S. BLEY